

Patented May 17, 1927.

1,629,110

# UNITED STATES PATENT OFFICE.

STANLEY P. LOVELL, OF BROCKTON, MASSACHUSETTS.

## STIFFENER FOR BOOTS AND SHOES AND COMPOUND USED THEREIN.

No Drawing. Application filed March 10, 1923, Serial No. 624,267. Renewed October 7, 1926.

The present invention relates to stiffeners such as are commonly employed for stiffening the toe and heel portions of the uppers of boots and shoes, and more particularly 5 to that type or class of stiffeners adapted to be softened by heat and to harden upon cooling.

Such stiffeners, as at present made, are 10 objectionable for various reasons. Some employ a stiffening compound containing rosin or similar crystalline substance, which not only renders the stiffener more or less brittle and liable to break when subjected to a sharp bending or crushing pressure, but 15 which gives off a dust when subjected to various operations incident to the preparation and use of the stiffeners, such as the dieing out, skiving, and trimming operations. This dust is unhealthful and annoying to the workmen, besides interfering 20 with the proper operation of the machine. Other stiffeners employ a stiffening compound of such nature that the work engaging instrumentalities of the various machines such as the needle of a shoe sewing 25 machine, the trimming knife of the upper or the vamp trimmer, the die cavity of the skiving machine, etc., tend to become gummy and sticky and difficulty is experienced 30 unless provision is made for lubricating or cleaning those parts during the operation of the machine.

Another objection to certain of the stiffeners heretofore produced has been the 35 high temperatures necessary properly to soften the stiffener and the small temperature range wherein the stiffener is in proper condition for manipulation and shaping.

It is the object of the present invention 40 to provide a stiffener suitable for box toes and counters of boots and shoes which shall avoid the above mentioned objections to prior stiffeners as well as other objections more specifically hereinafter referred to, 45 and with this object in view the present invention consists of the stiffener herein-after described and more particularly defined in the claims.

In carrying out the present invention I 50 may use as the base or body of the stiffener a fibrous material, such as felt, canton flannel, cheesecloth and the like, although preferably a cotton batting is employed since this gives superior results. Owing to 55 the structureless open character of this material and the sized or waxed or otherwise

finished surfaces, the stiffening compound with which the batting is impregnated is freely and uniformly absorbed, and a smooth, paper like surface is obtained which 60 permits the use of the stiffener on all grades of footwear without danger of printing or embossing the stiffener structure through the leather of the shoe, as is the case where a woven material is employed and the stiffener is in contact with a thin upper leather.

The stiffening material or compound which I employ consists of a lignite-extracted wax combined with a vegetable oil. Preferably I employ Montan wax, not only 70 on account of its cheapness but also on account of the improved character of the product although other waxes such as ozokerite, gilsonite, or grahamite may be 75 used.

Of the vegetable oils I prefer to use the oil of the soya bean. This oil can be procured in any desired quantity at low cost, and produces, when combined with one of the above mentioned waxes, and particularly 80 with Montan wax, a stiffening compound of a highly satisfactory character. Other vegetable oils, however, may be employed, such as cottonseed oil, corn oil, and less preferably, such oils as perilla bean oil, 85 arachis oil, cocoanut oil, olive oil and castor oil.

The siccative or drying oils, such as linseed oil and China wood oil, are not so well 90 adapted for use, not only on account of the characteristics of the compounds of these oils with the waxes above mentioned, but also because of their oxidizing action and liability to heating and spontaneous combustion.

In preparing the stiffening compound I have found satisfactory results are secured by heating Montan wax with soya bean oil, in the proportion of 64 pounds of wax to one gallon of oil, to a temperature of approximately 105 degrees centigrade, where the wax is dissolved in the oil and the two may be thoroughly mixed. The base or body of the cotton batting or other material is then impregnated with the stiffening compound in any suitable manner, such as by passing the material in the form of a web through the liquid stiffening compound, removing the excess compound by rollers or in any other manner, and permitting the web to cool and harden, after which it may be dried out and skived and otherwise pre-

pared for use as box toe or counter blanks, or any other purpose.

A stiffener as above described will soften at approximately 75 degrees centigrade, but the compound itself does not become liquid until 90 degrees or thereabouts is reached, thus giving a considerable range of temperature during which the stiffener may be manipulated and shaped to the last.

10 A feature of the present invention which is of importance is the control of flexibility of the stiffener by varying the proportion of wax and oil. Practically any desired degree of flexibility may be secured by increasing or diminishing the proportionate amount of oil. In prior stiffeners, particularly in those employing a stiffening compound consisting of several different substances, or containing a substance liable to variation in quality, great difficulty has been experienced in controlling or varying the flexibility. Owing to the substantially uniform and unvarying character of my ingredients, I am enabled to secure the desired flexibility with certainty and ease.

25 Re-heating of my improved stiffener, for any purpose, does not affect it. Furthermore, the compound is neutral in re-action, thus avoiding all possibility of damage to, or destruction of the adjacent parts of the shoe which may occur if rosin is employed in the stiffening compound, by reason of the release by the moisture or perspiration of the foot of such acids as colophonic and albeatic or uncombined alkalines from calcium or magnesium resinate.

The stiffening compound which I employ possesses a high adhesive quality which is of advantage particularly when the stiff-

ener is used for box toes, since it cements together some or all of the several parts of the shoe at the toe, such as the cap, doubler, lining, and stiffener itself. Inasmuch as the compound is free from stickiness when cold, there is no liability of the sock of the wearer of the shoe adhering to the lining.

Having thus described the present invention, what is claimed is:—

1. A stiffener for boots and shoes and the like, consisting of fibrous material impregnated with a stiffening compound comprising Montan wax and soya bean oil. 50

2. A stiffener for boots and shoes and the like, consisting of fibrous material impregnated with a stiffening compound comprising Montan wax and a vegetable oil. 55

3. A stiffener for boots and shoes and the like, consisting of fibrous material impregnated with a stiffening compound comprising a lignite-extracted wax and a vegetable oil. 60

4. A stiffener for boots and shoes and the like, consisting of fibrous material impregnated with a stiffening compound comprising a lignite-extracted wax and a semi- or non-siccative vegetable oil. 65

5. A stiffener for boots and shoes and the like, consisting of a cotton batting impregnated with Montan wax and a vegetable oil.

6. A stiffener blank for boots and shoes 70 and the like, consisting of cotton batting having finished surfaces impregnated with stiffening compound.

7. A stiffening compound for fibrous material consisting of Montan wax and soya 75 bean oil.

STANLEY P. LOVELL.

pared for use as box toe or counter blanks, or any other purpose.

A stiffener as above described will soften at approximately 75 degrees centigrade, but the compound itself does not become liquid until 90 degrees or thereabouts is reached, thus giving a considerable range of temperature during which the stiffener may be manipulated and shaped to the last.

A feature of the present invention which is of importance is the control of flexibility of the stiffener by varying the proportion of wax and oil. Practically any desired degree of flexibility may be secured by increasing or diminishing the proportionate amount of oil. In prior stiffeners, particularly in those employing a stiffening compound consisting of several different substances, or containing a substance liable to variation in quality, great difficulty has been experienced in controlling or varying the flexibility. Owing to the substantially uniform and unvarying character of my ingredients, I am enabled to secure the desired flexibility with certainty and ease.

Re-heating of my improved stiffener, for any purpose, does not affect it. Furthermore, the compound is neutral in re-action, thus avoiding all possibility of damage to, or destruction of the adjacent parts of the shoe which may occur if rosin is employed in the stiffening compound, by reason of the release by the moisture or perspiration of the foot of such acids as colophonic and albeatic or uncombined alkalines from calcium or magnesium resinate.

The stiffening compound which I employ possesses a high adhesive quality which is of advantage particularly when the stiff-

ener is used for box toes, since it cements together some or all of the several parts of the shoe at the toe, such as the cap, doubler, lining, and stiffener itself. Inasmuch as the compound is free from stickiness when cold, there is no liability of the sock of the wearer of the shoe adhering to the lining.

Having thus described the present invention, what is claimed is:—

1. A stiffener for boots and shoes and the like, consisting of fibrous material impregnated with a stiffening compound comprising Montan wax and soya bean oil. 50

2. A stiffener for boots and shoes and the like, consisting of fibrous material impregnated with a stiffening compound comprising Montan wax and a vegetable oil. 55

3. A stiffener for boots and shoes and the like, consisting of fibrous material impregnated with a stiffening compound comprising a lignite-extracted wax and a vegetable oil. 60

4. A stiffener for boots and shoes and the like, consisting of fibrous material impregnated with a stiffening compound comprising a lignite-extracted wax and a semi- or non-siccative vegetable oil. 65

5. A stiffener for boots and shoes and the like, consisting of a cotton batting impregnated with Montan wax and a vegetable oil.

6. A stiffener blank for boots and shoes and the like, consisting of cotton batting having finished surfaces impregnated with stiffening compound. 70

7. A stiffening compound for fibrous material consisting of Montan wax and soya bean oil. 75

STANLEY P. LOVELL.

#### CERTIFICATE OF CORRECTION.

Patent No. 1,629,110.

Granted May, 17, 1927, to

STANLEY P. LOVELL.

It is hereby certified that error appears in the above numbered patent requiring correction as follows: In the grant, name of inventor, for Stanley Lovell read Stanley P. Lovell; page 1 of the printed specification, line 112, for the word "dried" read "died"; and that the said Letters Patent should be read with these corrections therein that the same may conform to the record of the case in the Patent Office.

Signed and sealed this 7th day of June, A. D. 1927.

Seal.

M. J. Moore,  
Acting Commissioner of Patents.

CERTIFICATE OF CORRECTION.

Patent No. 1,629,110.

Granted May, 17, 1927, to

STANLEY P. LOVELL.

It is hereby certified that error appears in the above numbered patent requiring correction as follows: In the grant, name of inventor, for Stanley Lovell read Stanley P. Lovell; page 1 of the printed specification, line 112, for the word "dried" read "died"; and that the said Letters Patent should be read with these corrections therein that the same may conform to the record of the case in the Patent Office.

Signed and sealed this 7th day of June, A. D. 1927.

Seal.

M. J. Moore,  
Acting Commissioner of Patents.